

88 Patented May 4, 1943

2,318,574

## UNITED STATES PATENT OFFICE

2,318,574

CELLULAR STRUCTURAL MATERIAL AND  
METHOD OF PRODUCING THE SAME

Isaac Harter, New York, N. Y., Charles L. Norton,  
Boston, Mass., and Charles L. Norton, Jr., New  
York, N. Y., assignors to The Babcock & Wilcox  
Company, Newark, N. J., a corporation of New  
Jersey

No Drawing. Application January 26, 1939  
Serial No. 252,868

14 Claims.

(Cl. 106—111) 41

Our invention relates to improvements in methods of manufacturing light-weight heat resistant bodies having a high percentage of interstitial voids and adapted for use as thermal and sound insulating structures, and more particularly to methods of manufacturing products of the character described in which a solidifiable fluid mass is substantially increased in volume by being impregnated with air or gas filled voids or bubbles prior to setting.

The products made in accordance with our invention may be cellular, permeable, fibrous, refractory, of low thermal conductivity, or of good structural strength, or with more than one of these characteristics. When the product is both permeable and cellular, for example, it is especially useful as a high grade sound insulator.

The methods of forming voids or bubbles in a solidifiable fluid mass heretofore used or suggested in manufacturing methods of the character described can be classified as follows:

1. Air jet dispersion into the mass;
2. Mechanical agitation of a mass containing mucilaginous ingredients, to hold air bubbles entrapped from the surrounding atmosphere;
3. Inclusion of material in the mass effecting a chemical reaction when wet to generate gas bubbles; and
4. Performing a stable tenacious foam which is separately mixed into the mass.

The first three methods require the solidifiable fluid mass to be of a sufficiently heavy consistency, i. e. high viscosity, to mechanically retain the bubbles formed until the mass is molded and set. Such solidifiable fluid masses do not have a "foaming" characteristic, i. e. the capacity when of low viscosity and given proper mechanical agitation to form a stable structure under atmospheric conditions containing widely dispersed voids or bubbles. All of the above methods produce substantially similar end products, although the preformed foam method is superior in uniformity of dispersion, number and regulable size of the bubbles produced. These advantages of the preformed foam method are however offset from a commercial viewpoint by the lesser number of operating steps, with consequent savings in labor and machinery, of the other methods of bubble formation.

No way has been found to produce commercially a satisfactory product of the described character by mechanically agitating a solidifiable fluid mass of heavy consistency containing a foaming agent, such as soap, soap bark, saponin, flotation oils, or fatty acid sulphonates, which foaming agents are

quite satisfactory for use in a preformed foam process. Such foaming agents have limited ability to foam in the presence of a mixture of solid materials such as required for end products of the described character, as such mixtures usually include setting agents such as calcined gypsum or other calcium materials, since such materials tend to form insoluble calcium salts of the fatty acids of these agents. It has also been found that most of such foaming agents disadvantageously affect the action of the setting agent in the mass, with a consequent weakening of the end product.

Processes for manufacturing products such as wall board, sound insulators, thermal insulators, and refractories must permit low cost quantity production to be commercially useful; therefore any improvements tending to simplify, cheapen or reduce the manufacturing operations required are of substantial advantage in this field.

The general object of our invention is the provision of an improved method of manufacturing light-weight bodies of the character described, which is adapted for low cost quantity commercial production, and which permits a solidifiable fluid mass containing all of the materials required for the desired end product to be foamed in a single operation.

The various features of novelty which characterize our invention are pointed out with particularity in the claims annexed to and forming a part of this specification. For a better understanding of the invention, its operating advantages and specific objects attained by its use, reference should be had to the accompanying descriptive matter in which we have described various embodiments of our invention.

The best results are obtained in accordance with our invention by employing all of the following features in combination:

Firstly, instead of depending upon a solidifiable fluid mass of relatively high viscosity and no foaming characteristic, or performing a stable tenacious foam and subsequently mixing it with a solidifiable fluid mass, we employ a low viscosity solidifiable fluid mass having a foaming characteristic. By "low viscosity" we have in mind such viscosities as would not permit bubble retention by the mass if any of the first three bubble forming methods referred to above were used. With such viscosities the mass is more accurately characterized as "liquid" rather than simply "fluid" or "flowable." By using such solidifiable fluids of low viscosities characterized by a very high percentage of water in the mixture, end products with a higher percentage of voids are obtainable

due to the greater dispersion of the solid particles in a low viscosity mass, resulting in lighter weight products.

Secondly, instead of using as the foaming agent soap, saponin, flotation oils, fatty acid sulphonates or the like, we employ a synthetic surface active chemical which is a non-soap, which causes rapid wetting out of the solid particles in the mixture, which rapidly lowers the surface tension of the liquid, which is completely stable in the presence of alkaline compounds, such as lime or calcium hydroxide, and thus cannot interfere with either the foaming action or with the subsequent setting action of the hydraulic binder, and which also produces a bubble wall or film which is considerably stronger than those formed with foaming agents heretofore employed. With such a foaming agent, the solidifiable fluid mass can be said to have the "foaming" characteristic heretofore mentioned. We have discovered that the class of synthetic surface active chemicals consisting of sulphonated fatty alcohols, and particularly those forming alkyl sulphuric acid esters, i. e.  $C_nH_{2n+1}OSO_3Na$  in various physical forms and concentrations, form highly suitable foaming agents with the fluidity and agitation conditions used. Such synthetic surface active chemicals are sold commercially in the form of dry alkali metal salts of the sulphonated fatty alcohols. We have found that the dry sodium salt of the sulphuric ester of lauryl alcohol sold as a detergent under the trade name "Duponol" is a highly effective foaming agent under the operating conditions contemplated. The formula for this is  $C_{12}H_{25}O(SO_3)Na$ . The foaming agent employed is preferably incorporated in the mix in dry form mixed with the dry material, but could be incorporated in other ways.

Thirdly, a type of high speed mechanical agitation of the low viscosity solidifiable fluid mass is employed which results in a rapid formation of bubbles of a tenacious minutely fine stable character. We have found that high capacity high speed mixers with thin bladed beaters, such as used in the commercial production of mayonnaise, marshmallows, etc. are suitable for this operation. When a light-weight end product, such as insulating brick having a fired weight as low as 1 lb. per 101 cu. in. (standard fire brick size) is desired, the water and dry materials may be blended, either by adding the dry materials to the water or vice versa, so long as the desired high fluidity is attained, and a uniform high speed agitation employed. Preferably however, the dry materials are added to the water in view of the more rapid and uniform dispersion of the solid particles into the water thereby obtainable, while maintaining a high uniform rate of agitation. The total time required under commercial batch capacities for blending and agitating such mixtures in the mixing chamber and draining the foamed material into molds has been found to be less than one minute. The blending and foaming operations described are equally applicable for use in a continuous process.

When a heavier and stronger end product is desired requiring a proportion of dry materials to water such as would materially reduce the "foaming" characteristic of the mass, it has been found preferable to substantially decrease the rate of agitation during the latter part of the agitation period when the fluidity is lowest in order to minimize the escape of bubbles from the mix and thus avoid reduction of the percentage of voids therein. With all types of mixtures,

however, it is desirable to produce cavitation at the surface of the mass when starting the foaming operation and to that end the multiple blades of the beater are so situated relative to the surface of the mass that they are repeatedly being transferred from the air to the mass carrying down into the mass small quantities of air which later are divided up into smaller bubbles. It is usually desirable to have the beater blades totally immersed in the latter part of the agitating period. In no case is the agitation continued for a period beyond that which permits the mixture to be molded prior to setting.

An improved light-weight refractory insulating brick suitable for temperatures up to 2000° F. and having good load carrying properties has been made in accordance with our invention by first mixing the dry ingredients in the following proportions:

|                                                                                               | Per cent by weight  |
|-----------------------------------------------------------------------------------------------|---------------------|
| 20 Raw Georgia kaolin                                                                         | 50                  |
| Plaster of Paris                                                                              | 30                  |
| Grog or grindings from previously burned brick of the same character, no coarser than 35 mesh | 20                  |
| 25 Duponol                                                                                    | $\frac{1}{16}$ of 1 |

The dry mixture was then blended with water in a ratio of 10 parts of water to 12 parts of dry material by weight. The fluid mass was then mechanically agitated for periods of from thirty seconds to three minutes until the mass was impregnated with bubbles to an extent that the fired products were found to have a porosity between 80-90% by volume. Prior to setting, the mixture was run off into molds which were stripped as soon as the material was set hard enough to handle. The wet molded shapes were then fired in a suitable kiln. The brick temperature was raised in 1.5 hours to a temperature of 2200° F. and then held at that temperature for 1.5 hours. The kiln was operated with an oxidizing atmosphere throughout. The bricks produced varied in weight from 1-1.5 lbs. for standard size, with a thermal conductivity approximately one-sixth that of first quality fire brick.

An insulating brick of substantially similar properties was produced with the following formula:

|                                                                                               | Per cent by weight  |
|-----------------------------------------------------------------------------------------------|---------------------|
| 50 Raw Georgia kaolin                                                                         | 53.3                |
| Plaster of Paris                                                                              | 33.4                |
| Grog or grindings from previously burned brick of the same character, no coarser than 35 mesh | 9.2                 |
| 55 Pine sawdust (8 mesh)                                                                      | $\frac{1}{16}$ of 1 |
| Duponol                                                                                       | $\frac{1}{16}$ of 1 |

The formula distinguishes from the prior formula by the addition of a small amount of pine sawdust, which permits a more rapid burning cycle to be employed.

Insulating bricks of similar properties were also formed with an additional 20% of raw Georgia kaolin substituted for the grog in the first formula. Other refractory materials, such as magnesite, chrome, or zircon, may be used in lieu of kaolin. In all of these bricks, the bulk of the voids was very fine and of practically uniform dispersion, and generally globular in form. These voids in the finished product are surrounded by a net work of indurated foraminous partitions of the solid material which support the structure while rendering it permeable to a slight degree, and hence adapt it for sound as well as

heat insulation. In all of the above cases the brick is fired at a temperature and over a period sufficient for the clay and setting agent to provide an adequate ceramic bond.

A satisfactory plaster board has also been made according to our invention by combining a mixture of plaster of Paris and an amount of the described foaming agent in the proportion of  $\frac{1}{16}$  of 1% of the plaster of Paris by weight, with water in the ratio of one part of water to 1.43 parts of plaster of Paris by weight, mechanically agitating the same for a period of from 30 seconds to 5 minutes, depending upon water-temperature conditions, or until it is obvious no more air is being entrapped. In no case however, is the beating continued so long that there would be insufficient time to spread the material to a thickness of about  $\frac{1}{8}$  of an inch on building paper before setting occurs. A second sheet of building paper is then added in the usual manner. Hair or other fibrous material may be added to the mixture before agitation, if desired. When set the material is cut into sheets of suitable size.

In carrying out the foregoing processes, it will be found advantageous to use water at fairly elevated temperatures, that is to say from 100° to 180° F., as in such combinations of ingredients the use of warm water has been found to allow the use of smaller quantities of the foaming agent, than where water below 100° F. is used. Consequently for the same amount of the foaming agent with warm water, the volume of the mix can be increased more than 25% in a shorter time interval.

While the manufacture of several products in accordance with our invention has been described, it is nevertheless to be understood that in practicing the invention we may resort to modifications in both method and product so long as the same are within the scope of the appended claims defining the invention.

We claim:

1. The method of manufacturing light-weight insulating brick of high porosity which comprises forming a solidifiable mass of relatively low viscosity containing argillaceous material, plaster of Paris, water equal to at least 70% of the total weight of the other constituents, and an alkyl sulphuric acid ester foaming agent capable of rapidly wetting out the solid material in the mass, lowering the surface tension of the water, and stable in the presence of alkaline compounds, mechanically agitating the mass at a relatively high speed until the mass is foamed into a stable structure of substantially increased volume, molding the mass before setting, and firing the molded bodies.

2. The method of manufacturing light-weight non-metallic structural material of high porosity which comprises mechanically agitating a solidifiable fluid mass of relatively low viscosity containing argillaceous material, plaster of Paris, water equal to at least 70% of the total weight of the other constituents, and a small amount of fatty alcohol sulphate capable of rapidly wetting out the solid material in the mass, lowering the surface tension of the water, and stable in the process of alkaline compounds, until the mass is foamed into a stable structure of substantially increased volume, and shaping the foamed mass before setting.

3. The method of manufacturing light-weight insulating brick of high porosity which comprises blending a mixture of ceramic refractory material, plaster of Paris, a finely divided com-

bustible organic material, and an alkyl sulphuric acid ester stable in the presence of alkaline compounds, with an amount of water equal to at least 70% of the total weight of the other constituents to form a solidifiable mass of relatively low viscosity, and mechanically agitating the mass at a relatively high speed for a period shorter than the setting period of the mass and until the mass is foamed into a stable structure of substantially increased volume, molding the foamed mass before setting, and then firing to refractoriness.

4. The method of manufacturing insulating brick of relatively high porosity which comprises adding a mixture of argillaceous material, plaster of Paris, and an alkyl sulphuric acid ester stable in the presence of plaster of Paris, to sufficient water to form a solidifiable mass of progressively increasing viscosity during a major portion of the mixing operation, mechanically agitating the mass at a relatively high speed during the mixing operation until the mass is foamed into a stable structure of substantially increased volume, decreasing the rate of agitation as the viscosity of the mass increases, molding the mass before setting, and then firing the molded bodies.

5. The method of making a light-weight insulating brick of high porosity which comprises blending a dry mixture of argillaceous material, plaster of Paris, wood flour, and an alkyl sulphuric acid ester foaming agent, with sufficient warm water to form a solidifiable mass of relatively high fluidity while mechanically agitating the forming mass until a foamed stable structure of substantially increased volume is formed, molding the foamed mass before setting, and then firing the molded products, while containing substantially all of the water present after molding to a relatively high temperature during a relatively short burning cycle.

6. A structural burned ceramic product formed by burning a molded foamed water mixture of argillaceous material, calcined gypsum and a lauryl alcohol sulphate having after burning a density less than 25 lbs. per cubic foot.

7. A burnt ceramic cellular product formed by burning a foamed molded mixture of the approximate proportions:

|                                                                      |                                            |
|----------------------------------------------------------------------|--------------------------------------------|
| Raw Georgia kaolin                                                   | 50% by weight.                             |
| Plaster of Paris                                                     | 30% by weight.                             |
| Grog or grindings from previously burned brick of the same character | 20% by weight.                             |
| Alkyl sulphuric acid ester foaming agent                             | $\frac{1}{16}$ of 1% by weight.            |
| Water                                                                | 10 parts to 12 parts of dry mix by weight. |

8. A burnt ceramic cellular product formed by burning a foamed molded mixture of the approximate proportions:

|                                                                      |                                            |
|----------------------------------------------------------------------|--------------------------------------------|
| Raw Georgia kaolin                                                   | 53% by weight.                             |
| Plaster of Paris                                                     | 33% by weight.                             |
| Grog or grindings from previously burned brick of the same character | 9% by weight.                              |
| Pine sawdust                                                         | 4% by weight.                              |
| Alkyl sulphuric acid ester foaming agent                             | $\frac{1}{16}$ of 1% by weight.            |
| Water                                                                | 10 parts to 12 parts of dry mix by weight. |

9. A cellular unburned product formed by setting a foamed mixture of the approximate proportions:

Plaster of Paris 14.3 parts by weight.

Alkyl sulphuric acid ester foaming agent  $\frac{1}{6}$  of 1% by weight of the plaster of Paris.

Water 10 parts by weight.

10. The method of making a light-weight insulating refractory brick which comprises blending a dry mixture of argillaceous material, plaster of Paris, and an alkyl sulphuric acid ester foaming agent, with water equal to at least 70% of the total weight of the other constituents to form a solidifiable mass of relatively high fluidity while mechanically agitating the mass until a foamed stable structure of substantially increased volume is formed, molding the foamed mass before setting, and then subjecting the molded products while containing substantially all of the water present after molding to a relatively high temperature.

11. The method of making a light-weight insulating refractory brick which comprises blending a dry mixture of argillaceous material, plaster of Paris, a finely divided combustible organic material, and a sulphonated fatty alcohol foaming agent, with water equal to at least 70% of the total weight of the other constituents to form a solidifiable mass of relatively high fluidity while mechanically agitating the mass until a foamed stable structure of substantially increased volume is formed, molding the foamed mass before setting, and then firing the molded products when set sufficiently to permit handling and while con-

taining substantially all of the water present during the molding operation by subjecting the products to a relatively high temperature.

12. As a new article of manufacture, a burnt ceramic cellular product formed by burning a foamed molded shape formed from a mixture of dry materials including a ceramic refractory material, plaster of Paris and finely divided combustible organic material, the refractory material being over 50% and the hydraulic setting agent being over 20% by weight of the dry material, a small amount of an alkyl sulphuric acid ester foaming agent, and water equal to at least 70% of the total weight of the other constituents.

13. As a new article of manufacture, an insulating shape formed by burning a molded foamed mixture of ceramic refractory material, a quick-setting cementitious material, sawdust, an alkyl sulphuric acid ester foaming agent, and an amount of water equal to over 50% of the total weight of the other constituents of the mixture, and having after being fired a cellular porous stable indurated structure weighing less than 25 lbs. per cubic foot and a thermal conductivity approximately one-sixth that of first quality firebrick.

14. As a new article of manufacture, an insulating shape formed by burning a molded foamed mixture of argillaceous material, plaster of Paris, sawdust, an alkyl sulphuric acid ester foaming agent, and water approximating the weight of the other constituents and having after being fired a cellular porous stable indurated structure weighing less than 25 lbs. per cubic foot.

CHARLES L. NORTON,  
CHARLES L. NORTON, Jr.  
ISAAC HARTER.